

Oct. 15, 1946.

F. G. MANSON ET AL

2,409,370

FABRIC

Original Filed June 7, 1943



Inventor  
FRANK G. MANSON  
AND JAMES J. MASKEY

BY

*Louis A. Kline*

THEIR Attorney

## UNITED STATES PATENT OFFICE

2,409,370

## FABRIC

Frank G. Manson, Chicago, Ill., and James J. Maskey, Ferndale, Mich.

Original application June 7, 1943, Serial No. 489,959. Divided and this application April 25, 1945, Serial No. 590,272

4 Claims. (Cl. 139—420)

1

This is a division of our co-pending United States patent application Serial No. 489,959, which was filed on June 7, 1943, and which issued on September 4, 1945, as United States Patent No. 2,384,187.

This invention relates to a novel fabric for use in making parachute canopies and in particular relates to a fabric provided with a double "rip-stop" construction which provides extra strength to light-weight fabric.

The novel fabric from which panels for a parachute canopy may be cut is a strong, light-weight material having a network of heavy threads forming a primary "rip-stop" and having the primary "rip-stop" network sub-divided by a network of lighter threads forming a secondary "rip-stop," the spaces between the threads of the primary and secondary "rip-stop" networks being filled with enough still lighter warp and fill threads to provide the desired porosity for the parachute canopy in which the fabric is used.

It is an object of this invention, therefore, to provide a novel light-weight fabric from which panels of parachute canopies can be made.

Another object of the invention is to provide a novel light-weight fabric which is made strong by a network of primary and secondary "rip-stops."

With these and incidental objects in view, the invention consists in the provision of a novel fabric having superior qualities, the essential elements of which fabric are set forth in the appended claims, and a preferred form or embodiment of the fabric and an example of one use for the fabric are hereinafter disclosed with reference to the drawing which accompanies and forms a part of this specification.

In said drawing,

Fig. 1 illustrates a portion of the novel fabric and shows in particular the arrangement of the cross mesh heavy threads which are used to provide additional strength to the fabric and form the "rip-stop" construction therein.

Fig. 2 is a layout illustrating the manner in which the panels are cut from the novel fabric.

Fig. 3 is a plan view of a hemispherical parachute canopy, showing the arrangement of the panels and showing in particular the direction in which the threads of the fabric run in the different panels.

#### Description

Fig. 1 shows a portion of the novel fabric. This fabric may be made of any suitable material and contains a network of primary "rip-stops"

2

50 of heavy thread, as double, seventy denier thread, which primary "rip-stop" threads are spaced one inch apart and run at right angles to form a series of one-inch squares having two sides parallel to the selvage edge of the fabric. Each of the squares formed by the primary "rip-stops" 50 is divided into squares by secondary "rip-stops" 51 of lighter-weight thread, as triple, twenty denier thread. The threads of secondary "rip-stops" are spaced a quarter of an inch apart, and these squares, formed by the secondary "rip-stop" threads 51, are filled with still lighter-weight thread 52, as twenty denier thread, for warp and fill sufficient to give the desired porosity to the fabric.

The network of secondary "rip-stop" tends to limit any tear from extending past the quarter-inch squares formed thereby, but, even if the tear should break through a secondary "rip-stop," 20 it would be stopped by the heavier primary "rip-stop" before the tear could extend much more than an inch. Thus applicants have provided a fabric which is light in weight but which is made strong by the networks of primary and secondary "rip-stops."

As an example of the manner in which the novel fabric is used in making panels for parachute canopies, reference may be had to Fig. 2, which shows a portion of the fabric with the 30 selvage edges at 12 and 13. The shaded portions of Fig. 2 show diagrammatically the directions in which the threads run in the fabric. The fabric is cut along the lines 14, 15, and 16 to produce the panels 11, and the edges of the panels which are formed by these cuts are sealed or fused by heat if the fabric is made of thermoplastic material, and by the application of a suitable sealing compound if the fabric is made of other than a thermoplastic material, and 40 these edges, by being sealed, are made resistant to ravel and are the equivalent of selvage edges. In the panels thus cut, the "rip-stops" are not at right angles to the length of the panel but are at an angle thereto, as shown in Fig. 2.

45 The panels resulting from cutting the fabric according to the layout of Fig. 2 are joined as shown in Fig. 3, with the selvage edge of adjacent panels joined, as at 18, and the "rip-stop" threads in the adjacent panels, so joined, running in the same directions. The shaded portions of the panels in Fig. 3 show diagrammatically the direction in which the threads in the fabric run in the various adjacent panels.

55 Applicants, therefore, have provided a novel fabric which is particularly useful in the manu-

facture of parachute canopies because it is made very strong and resistant to rips by the provision of the primary and secondary "rip-stop" networks and at the same time is very light due to the fact that very light-weight thread can be used as warp and fill to fill up the spaces between the primary and secondary "rip-stop" networks sufficiently to give the fabric the porosity desired in the parachute canopy without making the fabric too heavy.

While the particular fabric herein shown and described is particularly adapted for use in the manufacture of parachute canopies, it is to be understood that it is not intended to confine the invention to the use of the fabric for this purpose or to the use of the particular weights of threads in the fabric as herein disclosed, for it is susceptible of other uses and can be formed of different weight threads all coming within the scope of the claims which follow.

What is claimed is:

1. A light-weight fabric from which parachute canopies may be made, consisting of a warp and fill of light-weight thread having therein a network of heavy thread to provide strength to the fabric and forming a primary "rip-stop" and a further network sub-dividing the primary "rip-stop," said further network being made of medium heavy threads to provide additional strength to the fabric and forming a secondary "rip-stop."

2. A light-weight fabric from which parachute canopies may be made, said fabric including a primary "rip-stop" network of heavy threads dividing the fabric into squares, a secondary

5

10

15

20

30

35

"rip-stop" network of lighter-weight threads sub-dividing the squares of the primary network into smaller squares, and a warp and fill of still lighter-weight thread filling the spaces between the threads of the primary and secondary "rip-stops"; said warp and fill being effective to give the fabric the desired porosity and at the same time allowing it to be very light in weight, while the primary and secondary "rip-stops" give the fabric strength without unduly adding to its weight.

3. A parachute fabric formed of a warp and fill of light-weight thread and having therein a network consisting of thread approximately seven times as heavy as those of the warp and fill to strengthen the fabric and to form a primary "rip-stop," and also having a further network sub-dividing the primary "rip-stop" and consisting of threads approximately three times as heavy as those of the warp and fill to provide further strength to the fabric and to form a secondary "rip-stop."

4. A light-weight parachute fabric including a primary "rip-stop" formed by a network of double, seventy denier threads running at right angles to each other and spaced apart to form one-inch squares, a secondary "rip-stop" formed by a network of triple, twenty denier threads spaced one-quarter of an inch apart to divide the one-inch primary "rip-stop" squares into quarter-inch squares, and a warp and fill of twenty denier thread between the threads forming the primary and secondary "rip-stops."

FRANK G. MANSON.

JAMES J. MASKEY.